

UNITED STATES PATENT OFFICE

2,293,419

# PROCESS FOR SOLUBILIZING LUBRICATING OIL ADDITIVES

**Paul R. Van Ess, Berkeley, Calif., assignor to Shell Development Company, San Francisco, Calif., a corporation of Delaware**

No Drawing. Application May 27, 1941,  
Serial No. 395,391

**6 Claims. (Cl. 252—35)**

This invention deals with compounded mineral lubricating oils and, more particularly, is concerned with a process for incorporating polyvalent metal salts of alkylated aromatic hydroxy carboxylic acids into mineral oils in which a decomposition product of said salts is used as a solubilizing agent.

It is known that in modern internal combustion engines, such as high-speed Diesel engines, aviation gasoline engines, etc., piston rings have a tendency to become stuck in the grooves; lacquer and/or carbon formation appear to be the principal reasons for this occurrence.

The addition of small amounts of certain metal salts of alkylated aromatic hydroxy monocarboxylic acids in which the carboxylic acid radical is attached directly to the ring, preferably in ortho position to the OH radical, when added to mineral oils is known to be especially effective in reducing ring-sticking tendencies of mineral oils. The aromatic hydroxy carboxylic acids may be mono- or poly-nuclear, suitable acids being, for example, alkyl salicylic, ortho hydroxy naphthoic or anthracene ortho hydroxy carboxylic acids. Suitable alkyl radicals are particularly those having three or more carbon atoms, such as *n* or isopropyl, butyl, amyl, cetyl wax, etc. radicals. One or several monocarboxylic alkyl radicals may be attached to the nucleus. Of the polyvalent metals which may be used to form the salts, magnesium, calcium, strontium, barium, zinc, tin, nickel, manganese, lead, copper, cobalt and aluminum are the most useful.

Many of the substances which are unusually useful as anti-ringsticking agents are difficult to dissolve in lubricating oils in effective quantities. To get such difficultly soluble compounds in solution, it has been necessary to heat mixtures of lubricating oils and their salts to temperatures of the order of 200° C. for a prolonged time, which often causes some deterioration of the oil. I have found that when dissolving these metallic salts at the elevated temperatures necessary for dissolution a portion of the salts decompose. The decomposition is believed to proceed according to the following equations, which postulate that the normal (or basic salt, as the case may be) is converted to an "inner ring" salt.



In general, at temperatures between about 160°–190° C., this reaction appears to be quite slow. Above about 190° C., however, it may become quite rapid.

5 It appears that the "inner ring" salts formed by  
this conversion are far more readily soluble in  
hydrocarbon oils than the "open" salts, and that  
dissolution of difficultly soluble salts by heating  
them to elevated temperatures is due to this ring  
10 closure. However, the conversion of all of the  
open to the inner ring salts is undesirable, because  
the latter have much poorer anti-ringsticking  
properties than the former. Reducing the tem-  
15 perature of this solution of the salts does not pre-  
vent the ring closure, in that the longer time  
required for dissolution at lower temperatures  
results in the formation of the ring products as  
well.

Now, I have discovered that the presence of relatively small amounts of the inner ring salt in a mineral oil greatly enhances the solubility of the more desirable open salts in this oil. Thus, by carefully controlling the time and temperature of the heating, it is possible to satisfactorily dissolve the desired open salt in a mineral oil without converting an excessive amount to the ring compound. However, in practice it is difficult to obtain the desired degree of partial conversion to the inner ring salt, since apparently the rate of conversion varies greatly depending on various factors, not all of which are known. For example, it is known that the salts of different metals are cyclized at widely different rates. Thus, when heating two 1% solutions of calcium and zinc di-isopropyl salicylates, respectively, in lubricating oil for 23 hours at 170° C., it was found that the percentages converted were 100% and 55% respectively.

40 The salts which most readily form the inner ring structures are those alkylated aromatic hydroxy monocarboxylic acid salts in which the carboxylic acid radical is in ortho position to the OH radical. Therefore, I prefer them for use as solubility agents for the dissolution of other alkylated aromatic ortho hydroxy mono carboxylates, 45 or of alkylated aromatic meta or para hydroxy mono carboxylates.

In order to facilitate control and to obtain a stable solution of one of the difficultly soluble salts with the minimum amount of conversion to the ring compound, I prefer to proceed as follows:

A solution of inner ring salt is first prepared by heating a mixture of a relatively small amount of the open salt and oil to between about 190°-53 200° C., substantially until  $\text{CO}_2$  evolution has ceased. The resulting solution is then cooled to below 190° C., and preferably between about 160°-60 170° C., whereupon additional amounts of the open salt are added which go in solution readily.

and rapidly substantially without evolution of CO<sub>2</sub>, i. e., without ring closure.

By this method it has, for example, been possible to dissolve in a lubricating oil as much as 30% of calcium di-isopropyl salicylate, less than 25% of which was converted to the ring compound. This solution was a suitable concentrate which could be blended with straight lubricating oil in any desired proportion to produce an anti-ringsticking lubricating oil containing, say, from .5%-.2.5% of the active open salt.

In general, it is desirable to convert at least about 10% and not more than 30%, and preferably from 15% to 25%, of the open to the inner ring compound. The percentage converted can be determined when measuring the amount of CO<sub>2</sub> evolved, or better yet, by determining the amounts of free alkyl phenol in the oil before and after the heating period.

If desired, one may first dissolve and convert to the ring compound a salt of one metal and thereafter dissolve a salt of another metal. This may have certain advantages in minimizing corrosiveness of the resulting finished oil.

If an amount of the salt in excess of that which is soluble at normal room temperatures is dissolved at the elevated temperature, it may be desirable to filter the oil after cooling in order to remove the excess.

It will be obvious to those skilled in the art that other additives, such as other anti-ringsticking agents, extreme pressure compounds, anti-wear agents, anti-oxidants, etc., can be added to the compounds prepared in accordance with my invention.

I claim as my invention:

1. In the process of dissolving in a mineral oil a difficultly soluble open salt combining a polyvalent metal with an aromatic hydroxy mono carboxylic acid, in which the carboxylic radical is directly connected to the aromatic nucleus to produce an anti-ringsticking lubricating oil, the improvement comprising heating a mineral oil containing a small amount of a salt formed by combining a polyvalent metal with an aromatic hydroxy mono carboxylic acid in which the car-

boxylic radical is attached directly to the aromatic nucleus under conditions to form an inner ring salt and thereafter dissolving a quantity of open salt in said mineral oil to produce a lubricant with anti-ringsticking properties.

2. In the process of dissolving in a mineral lubricating oil a difficultly soluble open salt combining a polyvalent metal with an aromatic ortho hydroxy mono carboxylic acid in which the carboxylic radical is directly attached to the aromatic nucleus to produce an anti-ringsticking lubricating oil, the improvement comprising heating a mixture of said oil and said salt to a temperature between 160°-200° C. under conditions to convert a minor portion only of said open salt to the corresponding inner ring salt and thereafter adding further quantities of the open salt under conditions to preclude the formation of CO<sub>2</sub>.

3. In the process of dissolving in a mineral oil a difficultly soluble open salt combining a polyvalent metal with an aromatic hydroxy mono carboxylic acid, in which the carboxylic radical is directly connected to the aromatic nucleus to produce an anti-ringsticking lubricating oil, the improvement comprising aiding the dissolution of said open salt by the addition of a concentrate prepared by heating a mineral oil containing a salt combining a polyvalent metal with an aromatic hydroxy mono carboxylic acid under conditions of time and temperature to liberate CO<sub>2</sub> and form an inner ring salt.

4. In the process of dissolving an open salt of calcium di-isopropyl salicylate in a mineral oil to produce an anti-ringsticking lubricant, the improvement comprising adding an inner ring salt of a polyvalent metal and an aromatic hydroxyl carboxylic acid as a solubilizing agent.

5. The process of claim 4 in which the added inner ring salt is the inner ring salt of calcium di-isopropyl salicylate.

6. The process of claim 4 in which the added inner ring salt is the inner ring salt of zinc di-isopropyl salicylate.

PAUL R. VAN ESS.